

# United States Patent

[11] 3,615,510

[72] Inventors **Joseph S. Yudelson;**  
Randall E. Mack, both of Rochester, N.Y.  
[21] Appl. No. **575,548**  
[22] Filed **Aug. 29, 1966**  
[45] Patented **Oct. 26, 1971**  
[73] Assignee **Eastman Kodak Company**  
Rochester, N.Y.

2,238,632 4/1941 Dersch ..... 96/109  
2,288,586 6/1942 Dersch ..... 96/109  
3,093,479 6/1963 Olivares ..... 96/50  
3,161,506 12/1964 Becker ..... 96/109  
3,177,237 4/1965 Muetterties ..... 260/448.2  
3,177,240 4/1965 Muetterties ..... 252/95  
3,179,517 4/1965 Tregillus ..... 96/50  
3,212,899 10/1965 Kennard ..... 96/95  
3,243,295 3/1966 Vogt ..... 96/61

[54] **SILVER HALIDE COMPLEXING AGENTS**  
16 Claims, No Drawings

*Primary Examiner*—Norman G. Torchin  
*Assistant Examiner*—Mary F. Kelley  
*Attorneys*—W. H. J. Kline and Bernard D. Wiese

[52] U.S. Cl. .... **96/61,**  
96/109  
[51] Int. Cl. .... **G03c 5/38,**  
G03c 1/34  
[50] Field of Search ..... 96/61, 109,  
95

[56] **References Cited**  
UNITED STATES PATENTS

3,347,675 11/1967 Henn et al. .... 96/67  
2,238,631 4/1941 Dersch ..... 96/109

**ABSTRACT:** Photographic silver halide can be stabilized with certain organic sulfonium, organic sulfoxonium, organic ammonium, organic phosphonium, organic boronium, and/or organic siliconium halides of mixtures of these. These can be employed in a photographic element, processing solution or processing web. They are useful in combination with a nonaqueous, low-melting solvent, e.g. succinimide, sulfamide, urea, or acetamide.

## SILVER HALIDE COMPLEXING AGENTS

This invention relates to silver halide complexing agents and in particular to the stabilization and fixing of silver halide sensitized photographic materials.

The usual procedure employed in the processing of light-sensitive silver halide photographic elements is development of the latent silver image followed by fixing to remove residual light-sensitive silver salts. If rapid processing of films and papers is desired and extreme permanence is not required, the unexposed silver halides may be left in the photograph and converted into compounds which are relatively inert to light, heat, and humidity. This type of rapid processing is known as stabilization and the criteria for judging its effectiveness are the stability of the resulting photographic image to moist incubation and light.

Many of the known stabilization processes utilize complexing agents which have serious limitations. Often, opaque complexes are formed or the complexing agent bleaches the silver image. Some of these complexing agents are activated by water and thus, such agents cannot be incorporated into aqueous gelatin-silver halide emulsions without adversely affecting the sensitometric characteristics of the emulsion or the light-sensitive layer. These water-activated complexing agents are not suitable for dry-processing techniques. In addition, few silver halide stabilizers have been found which operate satisfactorily in diffusion transfer processes. In this invention, silver halide complexing agents have been found which are free from these undesirable characteristics, and which can be used effectively to stabilize or fix a photographic element.

It is an object of this invention to provide photographic silver halide stabilization and fixing compositions which form stable, transparent silver halide complexes, and which can be in the form of either aqueous or nonaqueous solutions.

Another object is to provide a process for the stabilization of photographic images.

A further object is to provide a process for fixing photographic images which can employ aqueous or nonaqueous fixing baths.

Still another object is to provide a simplified process for the stabilization of a photographic silver halide element which requires only heating of the element.

A further object is to provide photographic silver halide stabilization compositions which can be employed in a photographic diffusion transfer process.

Still another object is to provide photographic silver halide elements containing a heat-activated stabilization composition which will enable such elements to be stabilized by heating alone.

A further object is to provide a class of silver salt complexing agents which have a slow rate of stabilization in cold aqueous solutions, but which will stabilize an exposed photographic element quite rapidly in hot aqueous solutions.

Still another object is to provide a class of silver halide complexing agents which are odorless, unusually stable to adverse changes of heat, light, and humidity, which have little tendency to bleach silver images, and which do not cause tack or stickiness in processed elements.

Another object is to provide a processing web containing silver halide complexing agents for processing photographic elements.

Still further objects will become apparent from the following specification and claims.

According to our invention, it has been found that light-sensitive silver halide photographic elements can be stabilized with a solution containing a stabilizing amount of a complexing agent selected from the group consisting of organic sulfonium halides, organic sulfoxonium halides, organic ammonium halides, organic phosphonium halides, organic boronium halides, organic siliconium halides, or mixtures thereof. Certain of these organic complexing agents may also be defined in accordance with the following formulas:



Wherein A is S; A' is N or P; X is a halide ion; R<sub>1</sub>, R<sub>2</sub> and R<sub>3</sub> are lower alkyl; R<sub>4</sub> is lower alkyl or aryl, e.g. phenyl.

In the above definition of R<sub>1</sub>–R<sub>6</sub>, amino includes substituted amino groups, hydroxy includes ether linkages, alkyl includes substituted alkyl groups, and aryl includes substituted aryl groups.

Especially preferred complexing agents falling within the above formula include tetraethylammonium bromide, 2-hydroxyethyltrimethylammonium bromide, tetraethylammonium chloride, ethyltrimethylammonium bromide, tetramethylammonium bromide, tetrapropylammonium iodide, methylamine hydrobromide, trimethylamine hydrobromide, tetraethylphosphonium bromide, n-butyl-triphenylphosphonium bromide, and trimethylsulfonium bromide. The complexing agents can be present in the solution in any amount which will effect stabilization and preferably comprise about 5 to about 40 percent by weight of the solution.

Solution of the silver halide complexing agent may be made either in water or in a suitable nonaqueous, low-melting solvent. The complexing agents of the invention have a slow rate of stabilization in cold, aqueous solutions, but when a photographic element is treated with a hot, aqueous solution of the complexing agent, rapid stabilization occurs.

Useful nonaqueous solvents which are liquid and will promote stabilization at room temperature include formamide, N,N-dimethylformamide, dimethylsulfoxide, and tetramethylene sulfone. Low-melting solvents, such as succinimide, sulfamide, acetamide, and urea, which are solids at room temperature, are also quite useful. They can be coated onto the photographic element or a separate processing web along with the stabilizer, so that stabilization can be effected merely by heating the element, or bringing it into contact with the hot processing web.

In a preferred embodiment of our invention, the silver halide complexing agents are incorporated in a low-melting, nonaqueous solvent, and a polymeric binder through which the melted solvent can diffuse. This mixture is coated as an image stabilization layer upon a light-sensitive photographic silver halide emulsion layer. The low-melting solvent is solid at room temperature, and the complexing agents contained therein are inactive. Upon heating, the solvent melts and allows diffusion of the complexing agent into the photographic emulsion layer where it reacts with unexposed silver halide to cause stabilization.

The combination of succinimide and tetraethylammonium bromide or tetraethylphosphonium bromide when used as a stabilizing composition has an exceptionally low tendency toward bleaching the silver image. Succinimide forms a clathrate which is extremely non deliquescent with tetraethylammonium bromide and with tetraethylphosphonium bromide, and thus fading is inhibited. Images stabilized with this composition do not fade as quickly as those fixed with alkali thiosulfates.

Quaternary ammonium compounds have been used in photographic processes of the prior art. In U.S. Pat. No. 3,093,479 of Olivares et al., granted June 11, 1963, fixing of a photographic image is followed by treatment with a solution of a quaternary ammonium halide to prevent image fading and overall yellowing and to protect the image from microbacterial deterioration. The quaternary salt, which is used in small concentrations (1-2 percent), combines with any residual thiosulfate from the fixing process, apparently forming an insoluble, immobile molecule which cannot react with aerial or residual sulfide ion. In our invention, quaternary ammonium compounds are used in larger amounts as silver halide complexing agents and react with the unexposed silver halide to

form stable complexes, probably of the type  $Q\oplus AgX_2\ominus$ . Thus, the quaternary salts act as stabilizers with the complexed silver halide either remaining in the element or being removed by washing.

U.S. Pat. Nos. 2,238,631 and U.S. Pat. No. 2,238,632 of Dersch et al., granted Apr. 15, 1941, and U.S. Pat. No. 2,288,586 of Dersch et al., granted June 30, 1942, describe the use of certain quaternary phosphonium iodides, ternary sulfonium iodides, and quaternary ammonium iodides to control yellow fog in photographic emulsions. These compounds are used in small amounts to prevent colloidal silver formed in the processing baths from forming a yellow deposit on the emulsion. In our invention, our compounds are used in larger amounts as complexing agents to prevent the printout of silver halide, an effect occurring after processing.

Two kinds of stabilizing agents which form complexes with silver halides are known in the prior art—those which produce insoluble silver halide complexes and those which produce soluble complexes. Insoluble silver halide complexes, which are usually opaque and, thus, generally not useful for stabilizing photographic film records, are formed from the reaction of thioglycolic acid, thiosalicylic acid, and similar mercapto compounds with silver halides. Alkali thiosulfates, alkali thiocyanates, thiourea, and certain thiourea derivatives convert silver halides into soluble complexes. The complexing agents of the invention constitute a new class of silver halide stabilizers quite unlike those of the prior art. They have a broad range of applications and avoid many of the limitations of the known stabilizers.

The stabilizing agents of our invention can be incorporated into photographic silver halide emulsion layers, or coated in separate layers contiguous to the emulsion layer. When incorporated into the emulsion layer, the stabilizing agents of the invention can be conveniently coated from aqueous solutions at or below room temperature without prestabilization of the emulsion. When these stabilizing agents are coated in a separate layer, solid, low-melting, nonaqueous solvents are used to provide a photographic element which may be stabilized merely by heating.

The silver halide complexing agents of the invention may also be utilized in stabilizing or fixing baths, using either nonaqueous solvents or hot water. A wide range of nonaqueous solvents may be used such as alcohols, ketones, nitriles, etc.

The processing solutions of the invention can also be incorporated into a separate processing web. Stabilization can then be effected by contacting the web having the solution imbibed therein with the exposed photographic element. Alternatively, a dry web containing the complexing agent and a low-melting solvent such as succinimide, sulfamide, urea or acetamide, can be contacted with a photographic element and heated to mobilize the complexing agent.

A developing agent may also be included in the photographic element or processing web which contains the stabilizing agent. The silver halide developing agents which may be used include those commonly known as silver halide reducing agents such as, for example 3-pyrazolidones, including 1-phenyl-3-pyrazolidone, 1-phenyl-4,4-dimethyl-pyrazolidone, etc., ascorbates, including sodium isoascorbate, p-phenylenediamine, hydroquinones, N-methyl-p-aminophenol sulfate, catechol, etc. Especially preferred developing agents are 1-phenyl-3-pyrazolidone and sodium isoascorbate. Thus, if a developer is added to an element or processing web which contains the complexing agents of the invention, development and stabilization can be achieved in a single processing step.

Another use of the silver halide complexing agents of the invention is in diffusion transfer processes. In such processes, a photographic element is first exposed and developed. The unexposed silver halide in the nonimage areas of the element are then complexed or stabilized and diffused to a receiving sheet containing active nuclei. In contact with these active nuclei, the silver complexes dissociate providing silver ions which can then be developed to a silver image on the receiving sheet. The complexing agents employed for this purpose must

be capable of picking up and transferring all of the unexposed silver halide, and more importantly, the resulting complex must dissociate in contact with the nuclei in the receiving sheet. Most silver halide stabilizers and complexing agents form complexes which will not readily or sufficiently dissociate in contact with the receiving sheet. The silver complexes formed with the stabilizing compositions of this invention dissociate readily in contact with the receiving sheet nuclei and thus provide an extremely useful diffusion transfer system.

When used to fix or stabilize a photographic image, the complexing agents of the invention need not be dissolved in only one solvent, but can also be dissolved in mixtures, complexes, or eutectics composed of several solvents. By a proper choice of solvents or mixtures of solvents, many variables in nonaqueous processing such as processing temperature, maximum density, fog level, and gamma can be adjusted as desired.

20 The photographic silver halide emulsions of the photographic elements which can be stabilized in this invention can be sensitized using any of the well-known techniques in emulsion making, for example, by digesting with naturally active 25 gelatin or various sulfur compounds and/or gold compounds. The emulsions can be sensitized with salts of noble metals of Group VIII of the Periodic Table which have an atomic weight greater than 100. The emulsions can be of the surface-sensitive or internally sensitive type. The emulsions can also contain speed-increasing addenda such as polyethylene glycols or thioether sensitizers.

20 The emulsions of the photographic elements which can be stabilized according to our invention can also contain conventional addenda such as gelatin plasticizers, hardeners and coating aids. These emulsions are useful in X-ray and other nonoptically sensitized emulsions, and can also be used in orthochromatic, panchromatic and infrared sensitive emulsions. The addenda can be added to the emulsion before or

40 after sensitizing dyes, if any, are used. Various silver halides can be used as the sensitive salt, such as silver bromide, silver iodide, silver chloride, or mixed silver halides such as silver chlorobromide or silver bromoiodide. The emulsions can be used in photographic elements intended for color photography, and thus can contain color-forming couplers, or used as emulsions to be developed by solutions containing couplers or other color-generating materials, or emulsions of the mixed-packet type, as disclosed by Godowsky, U.S. Pat. No. 50 2,698,794, or emulsions of the mixed-grain type, such as disclosed by Carroll et al., U.S. Pat. No. 2,592,243.

55 In the photographic elements which may be stabilized according to this invention, a wide variety of emulsion vehicles and dispersing agents for silver halide grains may be employed singly or in combination with each other, for example, gelatin, colloidal albumen, cellulose derivatives and synthetic resins, such as polyvinyl compounds. Examples of typical colloids which may be used are poly(vinyl alcohol), hydrolyzed 60 poly(vinyl acetate), hydrolyzed cellulose ester, water-soluble ethanolamine cellulose acetate, polyacrylamide, copolymers having a combined acrylamide content of 3-60 percent, copolymers of alkyl acrylate and acrylic acid, a vinyl alcohol copolymer containing urethane carboxylic acid groups or containing cyano-acetyl groups, or polymeric material which results from polymerizing a protein or saturated acrylated protein with a monomer having a vinyl group such as disclosed by Illingsworth, U.S. Pat. No. 2,852,382. Such polymeric addenda may be employed as latices or hydrosols in the preparation of the photographic emulsions of the photographic elements which may be stabilized according to our invention.

75 The following examples will further illustrate the invention but are not to be construed to limit it in any way.

75 The first three examples illustrate the effectiveness of the complexing agents of this invention as fixing agents.

## EXAMPLE 1

A 20 percent solution of 2-hydroxyethyltrimethylammonium bromide was made up in formamide. A sample of photographic paper which was made up of a gelatino-silver chloride emulsion (containing 77 mg. silver per square foot) was immersed in this bath for 1 minute at room temperature. This sample was washed in water for 5 minutes and analyzed for silver. The silver content was 1.6 mg. per square foot, indicating that with only 1 minute of treatment and 5 minutes' washing, practically all of the silver had been removed by this fixing composition.

## EXAMPLE 2

A 20 percent solution of 2-hydroxyethyltrimethylammonium bromide was made up in water. A sample of the silver chloride paper used in example 1 was immersed for 4 minutes at room temperature, washed in water for 5 minutes, and analyzed for silver. The silver content was 63 mg. per square foot. This demonstrates that the quaternary salt was a poor fixing agent in water at room temperature.

## EXAMPLE 3

The procedure of example 2 was repeated but with the quaternary salt solution at 90° C. and with an immersion time of 1 minute. The washed sample was analyzed for silver. The silver content was 2.5 mg. per square foot, indicating the 2-hydroxyethyltrimethylammonium bromide to be a good fixing agent in hot water.

## EXAMPLE 4

The following example illustrates the preparation and use of a photographic element containing a complexing agent of our invention.

## The following solution was prepared:

|                         |       |    |
|-------------------------|-------|----|
| A. Succinimide          | 30 g. | 40 |
| 1-Phenyl-3-pyrazolidone | 3 g.  |    |
| Sodium Isoascorbate     | 5 g.  |    |
| Water                   | 40 g. |    |

This solution was dispersed in 186 g. of 7 percent ethyl cellulose in toluene.

## The following solution was prepared next:

|                            |      |  |
|----------------------------|------|--|
| B. Succinimide             | 6 g. |  |
| Sulfamide                  | 2 g. |  |
| Tetrapropylammonium iodide | 6 g. |  |
| Water                      | 3 g. |  |

Solution B was dispersed in 186 g. of 7 percent ethyl cellulose in toluene.

The two dispersions, A and B, were mixed together in equal parts and then coated on paper having a gelatino-silver chloride emulsion using a 0.010-inch knife and dried. The coating was exposed to a line copy negative for 10 seconds (40 watt bulb) and heated on a 155° C. mandrel for 5 seconds. The print showed a good image ( $D_{max}$  0.4) and the background was pale yellow. The print was exposed to a fluorescent desk lamp for one week with no deterioration of the image and no darkening of the background.

When the quaternary salt was omitted from the "B" solution, no stabilization was observed and the print darkened very rapidly on exposure to room light.

## EXAMPLE 5

## The following solution was prepared:

|                            |         |    |
|----------------------------|---------|----|
| Succinimide                | 30 g.   | 70 |
| 1-Phenyl-3-pyrazolidone    | 3 g.    |    |
| Sodium Isoascorbate        | 5 g.    |    |
| Tetrapropylammonium iodide | 8 g.    |    |
| Water                      | 40 g. X |    |

This solution was dispersed in 186 g. of 7 percent ethyl cellulose in toluene.

The dispersion was coated (using a 0.008-inch knife) on paper having a gelatino-silver chloride emulsion. The coating was exposed to a line copy negative for 10 seconds (40 watt bulb) and heated on a 155° C. mandrel for 10 seconds. An image appeared during the first few seconds of heating. The sample was exposed to a fluorescent desk lamp (20 watt) at a distance of 6 inches for 24 hours with no deterioration of the image and no increase in fog level.

## EXAMPLE 6

## The following solution was prepared:

|                            |        |
|----------------------------|--------|
| Succinimide                | 15 g.  |
| 1-Phenyl-3-pyrazolidone    | 1.5 g. |
| Sodium Isoascorbate        | 2.5 g. |
| Tetraethylammonium bromide | 6.5 g. |
| Water                      | 15 g.  |

This solution was dispersed in 93 g. of 7 percent ethyl cellulose in toluene.

20 The dispersion was coated (0.008-inch knife) on paper having a gelatino-silver chloride emulsion and dried. The coating was exposed to a line copy negative for 10 seconds (40 watt bulb) and then heated on a 155° C. mandrel for 3 seconds. The developed image was exposed to a fluorescent desk lamp (20 watt) at a distance of 6 inches for 24 hours with no deterioration of the image and no increase in fog level.

## EXAMPLE 7

30 A sample from example 6 was stored at 50 percent relative humidity and 73° C. for 6 weeks. It was then exposed and heated at 155° C. for 3 seconds. The resulting developed and stabilized image showed approximately the same quality as that in example 6, indicating good shelf life of the coated paper.

## EXAMPLE 8

## The following solution was prepared:

|                                          |         |
|------------------------------------------|---------|
| Succinimide                              | 15.0 g. |
| Water                                    | 20.0 g. |
| 1-Phenyl-3-pyrazolidone                  | 1.5 g.  |
| Sodium Isoascorbate                      | 2.5 g.  |
| 2-Hydroxyethyltrimethylammonium chloride | 4.0 g.  |

45 This solution was dispersed in 93 g. of 7 percent ethyl cellulose in toluene.

The dispersion was coated (0.008-inch knife) on paper having a gelatino-silver chloride emulsion and dried. The coating was exposed to a line copy negative for 10 seconds (40 watt bulb) and heated on a 155° C. mandrel for 3 seconds. A gray, black image resulted with a yellow background. The print was stable to fluorescent light with no change in the image or background.

## EXAMPLE 9

55 The dispersion used in example 8 was coated (0.006-inch knife) on a substrate consisting of AgBr (30 mg. per square foot) which had been vacuum-deposited on paper support. The coating was exposed to a line copy negative for 20 seconds (40 watt bulb) and heated on a 155° C. mandrel for 3 seconds. A gray, black image appeared on a tan background. The print was stable to fluorescent light with no change in the image quality and no increase in fog.

## EXAMPLE 10

65 This example illustrates the use of quaternary ammonium halides in nonaqueous solvents as the silver halide complexing agent for a diffusion transfer process.

## The following solution was prepared:

|                                         |          |
|-----------------------------------------|----------|
| Sodium Isoascorbate                     | 3.0 g.   |
| 1-Phenyl-3-pyrazolidone                 | 0.5 g.   |
| 2-Hydroxyethyltrimethylammonium bromide | 5.0 g.   |
| Formamide                               | 50.0 ml. |

A piece of paper having a gelatino-silver chloride emulsion was exposed to a line copy negative for 30 seconds in a printing box (40 watt lamp). The solution was wiped over the surface of the photographic paper with a camel's hair brush and then a diffusion transfer receiving sheet was placed in face-to-face contact with the dampened paper. The sandwich was heated on a 140° C. mandrel for 2 seconds and the papers separated. A positive, brown-black image of that on the exposed paper was on the receiving sheet.

## EXAMPLE 11

The following solution was prepared:

|                            |         |
|----------------------------|---------|
| Succinimide                | 15.0 g. |
| Sodium Isoascorbate        | 2.5 g.  |
| 1-Phenyl-3-pyrazolidone    | 1.5 g.  |
| Tetraethylammonium bromide | 9.0 g.  |
| Water                      | 20.0 g. |

This solution was dispersed in 93 g. of 7 percent ethyl cellulose in toluene.

The dispersion was coated (0.004-inch knife) over a sheet of paper having a fogged, direct positive, silver chloride emulsion of the type in U.S. Pat. No. 2,541,472 and dried. It was then exposed for 45 seconds to a line copy negative using a number 2 Photoflood with a piece of yellow sheeting interspersed between the lamp and the negative. The coated paper was then heated on a 155° C. mandrel for 3 seconds and a positive reproduction of the "positive" image resulted. The print was stable to fluorescent light with no deterioration of the image and no increase in background.

## EXAMPLE 12

The following solution was prepared:

|                            |          |
|----------------------------|----------|
| Succinimide                | 10.0 g.  |
| Methane sulfonamide        | 5.0 g.   |
| Water                      | 20.0 ml. |
| 1-Phenyl-3-pyrazolidone    | 1.5 g.   |
| Sodium Isoascorbate        | 2.5 g.   |
| Tetraethylammonium bromide | 10.0 g.  |

This solution was dispersed in 93 g. of 7 percent ethyl cellulose in toluene.

The dispersion was coated (0.006-inch knife) over a sheet of paper having a gelatino-silver chloride emulsion and dried. It was then exposed to a line copy negative (10 seconds, 40 watt bulb) and heated on a 155° C. mandrel for three seconds. A brown image resulted with an off-white background. The paper was incubated at 100 percent relative humidity, 75° C., for 24 hours with no deterioration of the image and no increase in the background.

## EXAMPLE 13

The following solution was prepared:

|                            |        |
|----------------------------|--------|
| Succinimide                | 6.0 g. |
| Sulfamide                  | 2.0 g. |
| Water                      | 3.0 g. |
| Tetrapropylammonium iodide | 8.0 g. |

This solution was dispersed in 35 g. of 14 percent ethyl cellulose in toluene.

The dispersion was coated (0.004-inch knife) on a photographic paper which contained AgCl, gelatin, succinimide, 1-phenyl-4-methyl-3-pyrazolidone and sodium isoascorbate. The paper was then exposed to a line copy negative (30 seconds, 40 watt bulb) and heated on a 155° C. mandrel for 4 seconds. A black image resulted with a yellow background. The paper was exposed to fluorescent light for 24 hours with no deterioration of the image and no increase in background. This paper, when not coated with the dispersion, will give an excellent image after exposure and heating, but the background will darken on exposure to visible light.

## EXAMPLE 14

A silver halide emulsion was prepared as follows: (a) 14 g. of a silver chloride coagulum, which contains 15 g. of gelatin and one mole of silver in each 370 g. of emulsion, was dispersed in 100 g. of gelatin which also contained 7 g. of succinimide; (b) a solution was made as follows:

|                            |         |
|----------------------------|---------|
| Succinimide                | 15.0 g. |
| Water                      | 20.0 g. |
| 1-Phenyl-3-pyrazolidone    | 1.5 g.  |
| Sodium Isoascorbate        | 2.5 g.  |
| Tetrapropylammonium iodide | 8.0 g.  |

Ten parts of (a) were mixed with five parts of (b) and coated immediately on gelatin-subbed poly(ethylene terephthalate) film support. After drying, the coating was given an exposure of 5 seconds with a number 2 Photoflood (12-inch distance) and then heated for 10 seconds on a 155° C. mandrel. A developed and stabilized image resulted.

## EXAMPLE 15

The following solution was prepared:

|                                     |         |
|-------------------------------------|---------|
| Succinimide                         | 15.0 g. |
| Sodium Isoascorbate                 | 2.5 g.  |
| 1-Phenyl-3-pyrazolidone             | 1.5 g.  |
| n-Butyltriphenylphosphonium bromide | 10.0 g. |
| Water                               | 20.0 g. |

This solution was dispersed in 93 g. of 7 percent ethyl cellulose in toluene.

The dispersion was coated over paper having a gelatino-silver chloride emulsion using an 0.008-inch knife. The dried coating was exposed to a line image and heated for 5 seconds at 155° C. A developed and stabilized image resulted.

## EXAMPLE 16

The following solution was prepared:

|                               |          |
|-------------------------------|----------|
| Succinimide                   | 15.0 g.  |
| Sodium Isoascorbate           | 2.5 g.   |
| 1-Phenyl-3-pyrazolidone       | 1.5 g.   |
| Tetraethylphosphonium bromide | 9.0 g.   |
| Water                         | 20.0 ml. |

The solution was dispersed in 93 g. of 7 percent ethyl cellulose in toluene.

The dispersion was coated over paper having a gelatino-silver chloride emulsion using a 0.006-inch knife. The dried coating was exposed to a line image and heated at 140° C. for 3 seconds. A developed and stabilized image resulted.

## EXAMPLE 17

The following solution was prepared:

|                                    |          |
|------------------------------------|----------|
| Succinimide                        | 15.0 g.  |
| Sodium Isoascorbate                | 2.5 g.   |
| 1-Phenyl-3-pyrazolidone            | 1.5 g.   |
| Phenyltrimethylphosphonium bromide | 7.0 g.   |
| Water                              | 20.0 ml. |

This solution was dispersed in 93 g. of 7 percent ethyl cellulose in toluene.

The dispersion was coated over paper having a gelatino-silver chloride emulsion using a 0.008-inch knife. The dried coating was exposed to a line image and heated at 155° C. for 5 seconds. A developed and stabilized image resulted.

## EXAMPLE 18

The following solution was prepared:

|                            |          |
|----------------------------|----------|
| Succinimide                | 15.0 g.  |
| Sodium Isoascorbate        | 2.5 g.   |
| 1-Phenyl-3-pyrazolidone    | 1.5 g.   |
| Trimethylsulfonium bromide | 5.0 g.   |
| Water                      | 20.0 ml. |

This solution was dispersed in 93 g. of 7 percent ethyl cellulose in toluene.

The dispersion was coated over paper having a gelatino-silver chloride emulsion using a 0.006-inch knife. The dried coating was exposed to a line image and heated at 140° C. for 5 seconds. A developed and stabilized image resulted.

## EXAMPLE 19

The following solution was prepared:

|                                   |          |
|-----------------------------------|----------|
| Succinimide                       | 15.0 g.  |
| Sodium Isoascorbate               | 2.5 g.   |
| 1-Phenyl-3-pyrazolidone           | 1.5 g.   |
| Ethyl dimethylsulfoxonium bromide | 8.3 g.   |
| Water                             | 20.0 ml. |

This solution was dispersed in 93 g. of 7 percent ethyl cellulose in toluene. 15

The dispersion was coated over paper having a gelatino-silver chloride emulsion using a 0.004-inch knife. The dried coating was exposed to a line copy negative and heated at 155° C. for 3 seconds. A developed and stabilized image resulted. 20

## EXAMPLE 20 — Preparation of a Dry Processing Web

The following solution was prepared:

|                            |          |
|----------------------------|----------|
| Succinimide                | 10.0 g.  |
| Urea                       | 10.0 g.  |
| Sodium Isoascorbate        | 2.5 g.   |
| 1-Phenyl-3-pyrazolidone    | 1.5 g.   |
| Tetraethylammonium bromide | 10.0 g.  |
| Water                      | 20.0 ml. |

This solution was dispersed in 45 g. of a 15 percent toluene solution of cellulose acetate-butyrate. 30

The dispersion was coated over gel-subbed paper support using a 0.010-inch knife. A piece of paper having a gelatino-silver chloride emulsion was exposed to a line copy negative and then placed face-to-face with the paper web. The sandwich was heated on a 155° C. mandrel (paper side down) for 5 seconds. When separated, a developed and stabilized image was formed on the previously exposed paper. EXAMPLE 21

This example makes use of tropolone boron halides as complexing agents in nonaqueous systems. 40

Five grams (0.02 mole) of boron bromide was dissolved in 25 ml. of chloroform under a nitrogen atmosphere. A second solution consisting of 4.9 g. (0.04 mole) of tropolone in 120 ml. of chloroform was also prepared under nitrogen. The two solutions were mixed and refluxed for 3 hours. During this time a steady stream of nitrogen gas passed through the reaction mixture to carry off the HBr that is formed during the reaction. The reaction mixture was placed in an evaporating dish and left overnight in a dry box.

The product, a yellow solid, was recrystallized from water to give 5.6 g. of tropolone boron bromide.



| Analysis: | C    | H   | O     | B   | Br   |
|-----------|------|-----|-------|-----|------|
| Theo.     | 50.3 | 3.0 | 19.2  | 3.2 | 24.0 |
| Exp.      | 50.8 | 3.2 | 19.4* | 3.5 | 23.2 |

\*by difference

Tropolone boron bromide is soluble in water, formamide and molten succinimide. A 5 percent solution in water showed no tendency to dissolve silver chloride or silver bromide. A 5 percent solution in formamide (or molten succinimide) dissolved silver chloride and silver bromide very readily.

## EXAMPLE 22

This example makes use of tropolone silicon chloride as a silver halide complexing agent.

In an analogous procedure, silicon tetrachloride (4.6 g., 0.028 mole) in 50 ml. chloroform was added to a solution of tropolone (10 g., 0.08 mole) in 150 ml. of chloroform. After the addition, a rapid stream of nitrogen was passed through the mixture at reflux for 7 hours. After this time the evolution of HCl had ceased and a white solid separated. This was isolated by filtration and recrystallized from water to give 10.2 g. of tropolone silicon chloride ( $T_3Si^{115}Cl^{116}$ ).



Anal. Calcd. for  $T_3Si^{115}Cl^{116}$ :  
Found: C—48.2; H—2.9; Cl—6.8  
C—48.9; H—3.4; Cl—6.1

A 10 percent solution in water showed no tendency to dissolve silver chloride or silver bromide. A 10 percent solution in formamide (or molten succinimide) dissolved silver chloride.

## EXAMPLE 23

This example illustrates a quaternary halide-succinimide mixture for silver halide stabilizing processing at room temperature. A large amount of water was used to lower the crystallization point of the mixture.

The following solution can be used as a bath or as a surface application using a hopper or roller.

|                                               |           |
|-----------------------------------------------|-----------|
| Succinimide                                   | 26.0 g.   |
| Tetraethylammonium bromide                    | 20.0 g.   |
| Water                                         | 120.0 ml. |
| Dimethyl sulfoxide                            | 15.0 ml.  |
| Isooctylphenyl polyethoxyethanol (2% aqueous) | 6.0 ml.   |

55 A fine grain silver chloride paper was exposed and developed by a surface application of Kodak D-72 Developer (1:1) and then was stabilized by passing it over a roller dipped into the above stabilizing solution. After drying with warm air for 20–30 seconds, the samples were light-stable. Incubations for 3 days at 25° C., 75 percent relative humidity, showed no signs of image fading. Also, there was no sign of tackiness under the high humidity conditions.

60 Although the invention has been described in considerable detail with particular reference to certain preferred embodiments thereof, variations and modifications can be effected within the spirit and scope of the invention as described hereinbefore and as defined in the appended claims.

We claim:

65 1. A photographic silver halide stabilizing composition consisting essentially of a solution of an organic silver halide complexing agent in a silver halide stabilizing concentration of about 5 percent to about 40 percent by weight of said solution in a solvent which comprises formamide, dimethylsulfoxide, dimethylformamide, succinimide, sulfamide, urea or acetamide, said complexing agent being an organic sulfonium ha-

lide, an organic ammonium halide, an organic phosphonium halide, tropolone boronium halide, tropolone siliconium halide, or mixtures thereof.

2. The composition of claim 1 wherein said complexing agent is tetraethylammonium bromide, 2-hydroxy-ethyl-trimethylammonium bromide, tetrapropylammonium iodide, tetra-ethylphosphonium bromide, or trimethylsulfonium bromide.

3. The composition of claim 1 wherein the solvent is succinimide and the complexing agent is tetraethyl-ammonium bromide or tetraethylphosphonium bromide.

4. The composition of claim 1 wherein said complexing agent is tetraethylammonium bromide.

5. The composition of claim 1 which also contains a polymeric binder.

6. A process comprising developing a latent image in an exposed photographic silver halide element and stabilizing the undeveloped photographic silver halide, in said element with a solution consisting essentially of an organic silver halide complexing agent in a silver halide stabilizing concentration of about 5 to about 40 percent by weight of the solution; said complexing agent being an organic sulfonium halide, an organic ammonium halide, an organic phosphonium halide, a tropolone boronium halide, a tropolone siliconium halide, or mixtures thereof in water or a low-melting, nonaqueous solvent.

7. The process of claim 6 wherein complexed silver halide is removed from the element by washing.

8. The process of claim 6 wherein the solvent is formamide, dimethylformamide, dimethyl sulfoxide, succinimide, sulfamide, acetamide, urea, or water.

9. The process of claim 6 wherein said complexing agent is tetraethylammonium bromide, 2-hydroxyethyltri-methylammonium bromide, tetrapropylammonium iodide, tetraethylphosphonium bromide, or trimethylsulfonium bromide.

10. The process of claim 6 wherein said solution is heated to about 900° C. to about 155° C.

11. The process of claim 10 wherein the solvent is succinimide, sulfamide, urea, acetamide, or water.

12. The process of claim 10, wherein the solvent is succinimide and the complexing agent is tetraethylammonium bromide or tetraethylphosphonium bromide.

13. The process of claim 12 wherein said complexing agent is tetraethylammonium bromide.

14. A photographic silver halide stabilizing composition consisting essentially of a solution of an organic silver halide complexing agent, in a silver halide stabilizing concentration of about 5 percent to about 40 percent by weight of said solution, in a solvent which comprises a formamide, dimethylsulfoxide, dimethylformamide, Lmethylformamide, succinimide, Lsulfamide, urea or acetamide, said complexing agent being 10 (a) a compound of the formula:



wherein A is S; A' is N or P; R<sub>1</sub>, R<sub>2</sub> and R<sub>3</sub> are lower alkyl; R<sub>4</sub> is lower alkyl or phenyl; X is a halide ion;

- b. tropolone boronium halide; or
- c. tropolone siliconium halide.

15. The composition of claim 1 comprising a photographic silver halide developing agent.

16. A process comprising developing a latent image in an exposed photographic silver halide element and stabilizing the undeveloped photographic silver halide in said element, with a solution consisting essentially of an organic silver halide complexing agent, in a silver halide stabilizing concentration of about 5 percent to about 40 percent by weight of said solution, said complexing agent being (a) a compound of the formula:



wherein A is S; A' is P or N; R<sub>1</sub>, R<sub>2</sub> and R<sub>3</sub> are lower alkyl; R<sub>4</sub> is lower alkyl or phenyl; X is a halide ion;

- b. tropolone boronium halide; or
- c. tropolone siliconium halide, or mixtures thereof, in water or a low-melting, nonaqueous solvent.

UNITED STATES PATENT OFFICE  
CERTIFICATE OF CORRECTIONPatent No. 3,615,510 Dated October 26, 1971Inventor(s) Joseph S. Yudelson and Randall E. Mack

It is certified that error appears in the above-identified patent and that said Letters Patent are hereby corrected as shown below:

In the Abstract, line 4, "of mixtures" should read ---or mixtures---.

In Column 5, line 73, "40.0 g. X" should read ---40 g.----.

In Column 10, line 12, "(T<sub>3</sub>Si<sup>11</sup>Cl<sup>11</sup>6)" should read ---(T<sub>3</sub>Si<sup>+</sup>Cl<sup>-</sup>)---.

In Column 10, line 31, "T<sub>3</sub>Si<sup>+</sup>Cl<sup>1</sup>" should read ---T<sub>3</sub>Si<sup>+</sup>Cl<sup>-</sup>---.

In Column 10, line 51, after "polyethoxyethanol" insert ---surfactant---.

In Column 10, line 52, after "2% aqueous" insert ---solution)---.

In Column 10, line 56, after "it" insert ---twice---.

In the Claims:

In Column 11, line 6, "trimethlammonium" should read ---trimethylammonium---.

UNITED STATES PATENT OFFICE  
CERTIFICATE OF CORRECTION

Patent No. 3,615,510

Dated October 26, 1971

Inventor(s) Joseph S. Yudelson and Randall E. Mack

It is certified that error appears in the above-identified patent and that said Letters Patent are hereby corrected as shown below:

In Column 11, line 37, "900°C." should read  
---90°C.---.

In Column 12, line 8, "Imethylformamide" should read ---methylformamide---.

In Column 12, line 9, "Lsulfamide" should read  
---sulfamide---.

In Column 12, line 25, "underdeveloped" should read  
---undeveloped---.

Signed and sealed this 14th day of November 1972.

(SEAL)

Attest:

EDWARD M.FLETCHER, JR.  
Attesting Officer

ROBERT GOTTSCHALK  
Commissioner of Patents